

# UNITED STATES PATENT OFFICE.

CONRAD VARLEY GREENWOOD, OF BLUNDELLSANDS, NEAR LIVERPOOL, ENGLAND.

## TANNING.

1,349,150.

Specification of Letters Patent. Patented Aug. 10, 1920.

No Drawing.

Application filed July 28, 1915. Serial No. 42,339.

*To all whom it may concern:*

Be it known that I, CONRAD VARLEY GREENWOOD, a subject of the King of Great Britain, residing at Blundellsands, near Liverpool, in the county of Lancaster, in the Kingdom of England, have invented certain new and useful Improvements in Tanning, of which the following is a specification.

It is well known that in the tanning of skins for the production of leather by interaction of the skin substance with tannin in various forms, it is imperative to graduate these actions with various devices, generally by a succession of steps of increasing concentration of the extract or tannin. Hence the ordinary process is one of long duration requiring in the case of sole leather, *e. g.*, a period of several weeks or even months for the due carrying out of the successive treatment.

It is the object of the present invention to provide improved tanning methods embodying a more rapid process and producing a superlative quality of leather.

United States Patent No. 1105195 describes a process of producing a new or improved mucilaginous material. This specification suggested a possible application of the product in connection with tanning but it gave no details of such application, nor did it disclose the fact that the product exerted any action different to the action of tannin in the direction of speed of tanning or otherwise.

I have succeeded in devising processes employing hemicellulose *e. g.*, that obtained from the locust bean and similar colloids in such manner as to attain quite novel results.

It is well known that tannin in its various forms interacts with certain soluble colloidal carbohydrates to form compounds which are obtained as flocculent precipitates, or a more massive coagulum which retains much water in combination.

With certain carbohydrates of the hemicellulose class, the precipitant or coagulum has been observed to have the distinct characteristic of separating at lower temperatures in homogeneous opaque masses which are again liquefied on raising the temperature to form transparent highly viscous solutions. Such compounds or their manufacture are dealt with in the above-mentioned patent specification No. 1105195.

According to the processes which I have devised, it is possible to conduct tanning in such manner as to attain very considerable

advantages depending on the fact that the combination of tannin with such carbohydrates is of a weaker order than the combination of tannic acid with gelatin and nitrogenous colloids of the gelatin group. Hence when gelatin or a prepared animal skin is placed in contact with these compounds, both being in the normal stage of hydration and in presence of water, the superior attraction of the nitrogenous colloid exerts itself, and it combines with the tannin, the carbohydrates being displaced.

For obvious reasons, this process of combination by displacement is gradual, and hence the process of restrained tannage enables me to carry out the industrial process with very much increased rapidity.

The processes vary according to the circumstances and the following are typical methods of treatment:

(1) The skins or hides having been limed, unhaired, and flashed, are rounded and washed in a weak lime liquor in the ordinary way and are then ready for deliming.

This deliming is best carried out by suspending in a rectangular pit. A suitable deliming bath is made as follows:

For 60 butts, 1200 to 1500 gallons of water 8<sup>1</sup> 10 lbs. acetic, formic or hydrochloric or other suitable acid. The goods should be suspended for 24 hours.

It is extremely important that the deliming or acidifying should receive careful attention, and should be carried somewhat further than when tanning is by ordinary and older methods.

The goods after deliming, should be rinsed in water to remove the soluble lime salts and are then ready to tan.

For the preparation of the tanning material, the processes may vary according to the circumstances and the following are typical examples:—The hemicellulose is precipitated by means of the tanning extract or tannin and in some instances the mixture of the two materials is taken and used full strength. In others the coagulum or precipitate is allowed to separate. This is then dissolved in warm water and used as follows:

The goods are laid flat on a wooden board and are painted over on both sides with the aforesaid compound, making the application with a suitable flat brush. They are then laid perfectly flat in the bottom of a clean pit. An application of the aforesaid compound at least  $1\frac{1}{2}$  inches thick should be made between each pair of butts and same

laid on top of each other, flesh to flesh, the pit afterward being filled with the said solution to about 1 ft. above the uppermost pair of butts.

- 5 The goods should be left for 24 hours in this way and then carefully taken out on a sloping table leading into the pit so as to avoid any loss, the mixture thoroughly well stirred and the goods put back again, one at 10 a time. The goods are left in the mixture, strengthening if necessary by a further quantity of extract until a further penetration has been effected, this usually requiring 15 4 to 5 days when the goods on cutting will be found to be tanned completely through. The goods are now removed, the surplus material slicked off and are then washed in water at a temperature of about 45° centigrade until clean and then placed in layers 20 in the ordinary lay away pits, laying away in a 100° barkometer liquor with valones and myrobalans, or other suitable material. (2) The coagulum of hemicellulose tannic acid compound or mixture as already described may alternatively be used either full 25 strength or dissolved in water and added to the prepared hides or skins in a revolving drum. By this method the period of tanning is considerably reduced and the hides are 30 tanned completely through in the short space of about 24 hours.

(3) The more flocculent precipitant may be prepared, separated and collected, and then diffused in water in a suitable pit or bath, into which the prepared skins are placed and left at rest with occasional handling or strengthening if found necessary until the reaction is complete.

(4) The hemicellulose material may also be acted upon with synthetic tanning agents to form a suitable compound which would also be employed in the above described manner. Alternatively, any suitable colloidal body may be used in place of the hemicellulose material for the purpose of interaction with natural or synthetic tanning agents provided that the result is such as to exhibit the restraining action above described.

I use the words "restraining colloid" to denote a colloid preferably of the hemicellulose class which, exhibiting the property of being able to combine with the tannin in competition with the hide substance, is thus able to exert the above described restraining or inhibiting action on the process of tanning.

In other words, in its broadest form the invention covers processes of tanning by "organic" materials in which the process is considerably accelerated by thus designating employing a colloidal restraining agent in conjunction with such tanning. The best colloidal materials appear to be the soluble hemicelluloses above described but the in-

vention also extends to other colloidal materials exhibiting similar properties.

I declare that what I claim is:—

1. A process of tanning in which a hemicellulose restraining colloid is employed under conditions so chosen that a tanning effect is obtained at least equal to that which would be obtained without the use of the restraining colloid but in a considerably less time. 70

2. A process of tanning in which a restraining colloid is employed in conjunction with a tanning solution which is stronger than would be possible if the restraining colloid were not employed so that the same 80 tanning effect is obtained as in the usual tanning processes but in a very much shorter time. 75

3. A process of tanning in which a hemicellulose obtained from the locust bean is 85 employed in conjunction with a stronger tanning solution than usual so that at least as good a tanning effect is obtained but the time is considerably shortened.

4. A process of tanning sole leather in 90 which the butts are coated with a mucilaginous paste consisting of a compound of hemicellulose and tannin and said butts are immersed in a liquor containing the same ingredients in solution. 95

5. A process of tanning in which the goods are treated with a compound composed of vegetable restraining colloid and a tannin, and immersing the goods thus treated in a liquor containing the same ingredients in solution. 100

6. The herein described process of tanning which consists in employing an abnormally strong tanning solution in conjunction with a restraining colloid of vegetable origin under such conditions that the same 105 tanning effect is obtained as in the usual tanning process but in a very much shorter period of time.

7. The herein described process of tanning which consists in employing an abnormally strong tanning solution in conjunction with a restraining substance susceptible of combining with the tannin of the solution and thereafter gradually imparting the 115 same to the leather or hide being treated.

8. A process of tanning in which the goods are first treated with a vegetable restraining colloid and subsequently treated with a tanning agent of such strength as 120 would injure the goods except for the presence of the restraining colloid.

In witness whereof, I have hereunto signed my name this 15th day of July 1915, in the presence of two subscribing witnesses. 125

CONRAD VARLEY GREENWOOD.

Witnesses:

H. SHORTRIDGE,  
W. H. BEESTON.